

# UNITED STATES PATENT OFFICE.

DAVID FOSTER GOULD, OF NEWARK, NEW JERSEY, ASSIGNOR TO GENERAL LEAD BATTERIES COMPANY, A CORPORATION OF DELAWARE.

## SEPARATOR FOR STORAGE BATTERIES AND METHOD OF MAKING.

1,390,355.

Specification of Letters Patent. Patented Sept. 13, 1921.

No Drawing.

Application filed August 24, 1916. Serial No. 116,594.

To all whom it may concern:

Be it known that I, DAVID FOSTER GOULD, a citizen of United States, residing at Newark, county of Essex, and State of New Jersey, have invented new and useful Improvements in Separators for Storage Batteries and Methods of Making, of which the following is a specification.

This invention relates to means for spacing or holding apart the plates of storage batteries, such means being commonly known as separators, and more particularly it relates to such devices made from wood.

The invention has for one object the provision of a method for treating sheets of wood for the use as indicated, said method being relatively simple, inexpensive and rapid and capable of producing separators of the proper requirements *i. e.* porosity (so as to increase the fluid passages through the wood, thereby allowing diffusion of the acid through the cell and affording enlarged paths for the electric current so that the resistance is reduced), long life under working conditions in a battery and a low content of the various gums, resins, coloring matters and substances of similar nature which occur in wood and which may be called impurities of the wood.

A further object of the invention is the provision of a separator for storage batteries which shall have the characteristics named above.

Certain woods as for instance cypress, Douglas fir, white cedar, red wood and like woods contain in their natural state no substance in sufficient quantities to injure the positive plates of a battery when in use, and I have found that such woods require only to have their porosity increased to a suitable degree in order to form serviceable and substantial battery separators. In these woods there is a sort of incrusted matter on the true wood fibers which is composed principally of gums, resins, coloring matters and like substances. This matter occupies the spaces between the fibers of the wood. If the separators are placed in the battery with the wood in its natural state, the incrusted matters during the operation of the battery are oxidized forming carbon-dioxide and water as the main products. By removing the incrusted matters before using the separator in a battery, advantages are obtained, in addition to that of increasing the porosity as already referred to, among which may be

mentioned the increased efficiency of the battery especially during the first discharges caused by the prevention of the loss of electrical energy which takes place when part of the current is used up in oxidizing the incrusted matters. The increasing of the porosity increases the ampere hour capacity of the battery as the internal resistance of the battery is reduced and it also aids the diffusion of the acid to make up for the weakening of the electrolyte in the pores of the plates. The treatment required for the separator is one which will remove the substance named above and which clog the pores of the wood, but which will not attack the wood fiber proper to any appreciable extent, leaving the wood structurally strong and yet porous.

Boiling the wood in water or treating it with steam will dissolve out some of the insulating compounds between the fibers of the wood but does not remove the clogging material referred to so as to give that porosity and other advantages required for the most efficient operation of the battery.

Treatment of the wood with solutions of caustic soda also fail to give the desired character of separator. Such treatment mellows and softens the fiber and causes the material to swell into a soft and structurally weak mass.

I have found that the substances named above as impurities may be effectively removed by treatment in a dilute solution of a sulfite which may be an acid sulfite. The bodies of wood shaped as separators are immersed in such a solution and allowed to remain for a length of time and at a temperature which depends upon the kind of wood used and the degree of porosity desired. An example of my invention and treatment is to soak the wood in a 5% solution of sodium sulfite at 180° Fahrenheit for six hours, allow the solution to cool and stand for a further period of about twelve hours after which the excess sulfite is removed with water. During the second period the products which are formed by the action of the sulfite diffuse out of the wood. The exact strength of the solution used and the duration and temperature of the treatment are factors which depend on the kind and condition of the wood, the porosity desired and the time available. In order to shorten the time of treatment the wood may be treated with a stronger solution than 5% under

pressure in a digester. Other sulfites or acid sulfites may be substituted for the sodium sulfite as for example potassium sulfite and calcium acid sulfite. The strength of the 5 solution used is such that the various clogging matters are removed without the wood fiber itself being appreciably attacked, this leaving the wood fiber of the separator structurally strong. The wood fibers are more 10 wiry and stronger than by the other methods of treatment referred to. For instance the caustic soda method softens and mellows the fiber while fibers of the separator produced by the present invention are harsh 15 and strong, the difference between the fibers in the two cases corresponding roughly to the difference between linen and cotton fibers.

While the invention has been illustrated 20 by detailing an example of the process and examples of the separators produced, both the method and the product may be varied without departing from the spirit of the invention which is not therefore limited to the 25 details of the examples given.

What I claim as new and desire to secure by Letters Patent is:—

1. The process of preparing battery separators which consists in shaping wood containing no substance in sufficient quantity to injure the positive battery plate, into the 30 form of a separator, increasing the fluid passages through the wood by the removal of gums, resins and other substances, not an 35 integral part of the true wood fiber, by immersing in a solution of a sulfite and heating the solution to such temperature and for such time as produces the porosity desired, the wood of the finished separator containing a small quantity of 40 gum, resin and other substances not an integral part of the true wood fiber, relatively to those naturally existing in the wood.

substances, not an integral part of the true wood fiber, relative to those naturally existing in the wood.

2. The process of preparing battery separators which consists in shaping wood containing no substance in sufficient quantity to injure the positive battery plate, increasing the size of the fluid passages through the wood by the removal of gums, resins and other substances, not an integral part of the 45 true wood fiber, by soaking the wood in a five (5%) per cent. solution of sodium sulfite at a temperature of 180° Fahrenheit for six (6) hours, allowing the solution to stand and cool for twelve (12) hours and removing the excess sulfite with water, the wood of the finished separator containing a small quantity of gums, resins and other substances, not an integral part of the true wood fiber, relative to those naturally existing in 50 the wood.

3. A battery separator which consists of a wood naturally containing no substances in sufficient quantity to injure the positive battery plates, the fluid passages through 65 the wood being relatively increased in size by the removal of gums, resins and other substances, not an integral part of the true wood fiber, by immersing in a solution of a sulfite and heating the solution to such temperature and for such time as produces the porosity desired, the wood of the finished separator containing a small quantity of 70 gum, resins and other substances not an integral part of the true wood fiber, relatively to those naturally existing in the wood.

In testimony whereof, I have signed my name to this specification this 23rd day of August, 1916.

DAVID FOSTER GOULD.